

## 1

3,468,121  
METHOD OF PRODUCING SPRINKLY COLORED  
FIBROUS MATERIAL

Hirotaka Nakashima, Katsunosuke Maeda, Togo  
Fukunaga, Satoru Suzuki, and Kenichiro Matsuoka,  
Mishima-shi, Japan, assignors to Toyo Rayon  
Kabushiki Kaisha, Tokyo, Japan, a corporation of  
Japan

No Drawing. Filed Aug. 7, 1967, Ser. No. 658,660  
Claims priority, application Japan, Aug. 9, 1966,  
41/51,980; Nov. 17, 1966, 41/75,614  
Int. Cl. D02g 3/36, 3/02

U.S. CL. 57—164

6 Claims

## ABSTRACT OF THE DISCLOSURE

Methods of producing sprinkly colored yarns or yarns capable of being so dyed, which comprises gathering together, drawing and twisting together yarns (A) and (B) wherein yarn (B) is one which either has been dope-dyed or has a higher dyeability than yarn (A), with the proviso that the yarns (A) and (B) are those which, upon being drawn, possess the properties that the elongation of the latter is 3-9% greater than that of the former and the denier ratio of the former to the latter ranges between 1:1 and 3:1.

This invention relates to a method of producing sprinkly colored fibrous materials. More particularly, the invention relates to a method of producing yarns and fabrics of sprinkly colored synthetic fibers or yarns and fabrics having the potentiality of being dyed to such a tone.

Heretofore, as one of the methods of producing sprinkly colored yarn, there is known that in which a twisted yarn dyed to a certain shade and that which is either undyed or dyed to another shade are combined and crimped with a crimping apparatus. Another method is that in which twisted yarns composed of different classes of material fibers are combined and crimped, after which the composite yarn is dyed with a dyestuff which dyes one of the material fibers but not the other. However, in these methods, the initial twist possessed by each of the original yarns to be combined and the twist resulting from their untwisting have a great effect such that the composite product has the character of a plied yarn. Hence, the different yarns are not present evenly in this composite yarn or in a fabric knitted or woven therefrom but rather in a discrete fashion, with the consequence that spottiness in the pattern occurs and the sprinkly colored pattern displayed is of a confused pitch. As still another method, one in which the drawing and twisting together of different classes of undrawn multifilament yarns are carried out simultaneously has been attempted. In a method such as this, only unsatisfactory products could be obtained however, because of the difference in drawability between the different classes of multifilament yarns which gave rise to either filament breaks during the processes of twisting the yarns together or to slacks and strains to result in nonuniformity of the twist.

As a result of much investigation with a view to eliminating the various drawbacks of the conventional methods such as hereinabove described, we found that in gathering together, drawing and twisting together an undrawn synthetic multifilament yarn and a dope dyed undrawn synthetic multifilament yarn, very desirable sprinkly colored yarns could be obtained by specifying, as hereinafter to be described, the elongation possessed by the two multifilament yarns and the denier ratio

## 2

thereof. The so obtained yarn has a beautiful appearance as well as the feature that it is not easily discolored by means of abrasion. It was also found that a yarn capable of being dyed a sprinkly tone could be obtained in similar manner from an undyed, undrawn synthetic multifilament yarn and an undrawn synthetic multifilament yarn having a higher dyeability than that of the former.

It is therefore an object of this invention to provide a method of producing from undrawn synthetic multifilament yarns sprinkly colored yarns of uniform sprinkly colored pattern or yarns which can be so dyed, the production of which is accomplished evenly without giving rise to hardly any filament breaks or accompaniment of slacks or strains in the filaments.

One mode of this invention consists of a method of producing sprinkly colored yarns, which comprises gathering together an undrawn synthetic multifilament yarn (A) and a dope-dyed undrawn synthetic multifilament yarn (B) and thereafter drawing and twisting the yarns together, with the proviso that the yarns (A) and (B) are those which, upon being drawn, possess the properties that the elongation of the latter is 3-9% greater than that of the former and the denier ratio of the former to the latter is 1:1-3:1.

Another mode of the invention consists of a method of producing yarns which can be dyed to a sprinkly colored pattern, which comprises gathering together an undrawn synthetic multifilament yarn (A) and an undrawn synthetic multifilament yarn (B) of higher dyeability than that of yarn (A) and thereafter drawing and twisting the yarns together, with the proviso that the yarns (A) and (B) are those which, upon being drawn, possess the properties that the elongation of the latter is 3-9% greater than the former and the denier ratio of the former to the latter is 1:1-3:1.

For a better understanding of this invention, it will be more fully described hereinafter with reference being had to the results of experiments which were conducted during our investigation.

First, as a typical example, the drawing and twisting together of a white polyethylene terephthalate multifilament yarn and a dope-dyed polyethylene terephthalate multifilament yarn will be described. The term "white yarn," as here used, denotes an undyed white colored yarn which may or may not contain a small quantity of titanium dioxide, while the term "dope dye yarn" denotes a colored yarn which has been obtained by spinning a molten polymer containing a pigment. In making a yarn by drawing these two yarns and twisting them together, the main troubles that are encountered are: (a) that filament breaks occur or slacks and strains occur in the filaments during the yarn making process; and (b) that there is a difference in the sprinkly colored tones between each of the woundup pirls.

One example of the results that were obtained by an experiment of ours when we were investigating into the cause of these troubles is presented below.

Polyethylene terephthalate having an inherent viscosity of 0.60 and containing 2% of titanium dioxide as a delustrant and polyethylene terephthalate having an intrinsic viscosity of 0.60 and containing 3.2% of a blue pigment were each separately melt-spun under their respective optimum melt-spinning conditions at a speed of 1000 meters per minute at 20 grams per minute to obtain respectively a white undrawn multifilament yarn and a dope-dyed undrawn multifilament yarn. Three classes of yarns were made by drawing and twisting these two multifilaments alone as well as together. The elongation of these two multifilaments, after drawing, was in either case 26% and the denier of all three product yarns was 50 deniers. The

results obtained after spinning for 24 hours using 150 spindles are shown in Table I.

TABLE I

| Yarn                      | Number of spindles $\times$ time, hr. | Tenacity, g./d. | Elongation, percent | Number of spindles in which slacks occurred | Number of spindles in which breaks (including fluffs) occurred in filament |
|---------------------------|---------------------------------------|-----------------|---------------------|---------------------------------------------|----------------------------------------------------------------------------|
| Composite yarn            | 150 $\times$ 24                       | 4.7             | 24                  | 1 5<br>2 38                                 | 1 29<br>2 3                                                                |
| White yarn alone          | 150 $\times$ 24                       | 4.8             | 26                  | None                                        | 1                                                                          |
| Dope-dyed blue yarn alone | 150 $\times$ 24                       | 4.8             | 26                  | None                                        | 1                                                                          |

<sup>1</sup> Blue yarn.

<sup>2</sup> White yarn.

As apparent from the results given in the foregoing table, the drawability of the yarn is very inferior in the case of that consisting of two components twisted together as compared with that of the two components when used alone. From these results, it is seen that in the composite twisted yarn the slacks of the white yarn and the filament breaks of the dope-dyed blue yarn are very numerous. The cause for this is believed to be due to the fact that the rate of shrinkage of the dope-dyed blue yarn immediately prior to its being wound up on a pinc is greater than that of the white yarn. Namely,

less if the difference in the elongations (percent) between the white yarn and the dope-dyed blue yarn is 3-9%.

Further, white multifilament yarns having the five elongation levels of 10, 15, 20, 25 and 30% and, correspondingly, 55 classes of dope-dyed blue multifilament yarns whose elongations were higher by 1% to 11% in 1% increments were made, and these white and blue yarns were combined accordingly and twisted together. The twisting together of the yarns was carried out for 24 hours with 150 spindles. The results of 8250 spindles are presented in Table III below. The number of slacks and filament breaks in the table are the number of occurrences in one spindle.

TABLE III

| Difference in elongation (percent) between the dope-dyed blue yarn and white yarn | Number of slacks |      |      | Number of filament breaks |      |      |
|-----------------------------------------------------------------------------------|------------------|------|------|---------------------------|------|------|
|                                                                                   | X<br>(average)   | Max. | Min. | X<br>(average)            | Max. | Min. |
| 1                                                                                 | 16               | 21   | 3    | 13                        | 20   | 0    |
| 2                                                                                 | 9                | 17   | 0    | 8                         | 13   | 2    |
| 3                                                                                 | 3                | 5    | 0    | 2                         | 6    | 0    |
| 4                                                                                 | 1                | 3    | 0    | 2                         | 4    | 2    |
| 5                                                                                 | 2                | 4    | 0    | 1                         | 2    | 0    |
| 6                                                                                 | 1                | 2    | 0    | 3                         | 5    | 7    |
| 7                                                                                 | 3                | 5    | 0    | 1                         | 3    | 0    |
| 8                                                                                 | 2                | 4    | 0    | 2                         | 6    | 0    |
| 9                                                                                 | 5                | 8    | 1    | 4                         | 7    | 0    |
| 10                                                                                | 19               | 28   | 11   | 17                        | 21   | 0    |
| 11                                                                                | 45               | 65   | 34   | 29                        | 41   | 0    |

since the drawing tension prior to the draw rolls is greater than the tension between the draw rolls and the windup, the yarn becomes somewhat relaxed subsequent to the draw rolls and the difference in the shrinkage of the white yarn and the dope-dyed blue yarn in this state worsens the drawability. We found that for eliminating the appearance of this trouble which was ascribable to the difference in the relaxation and shrinkage of the two components under identical drawing conditions it was necessary to use a yarn of higher elongation in the case of that having a higher relaxation and shrinkage, i.e., to use as the blue yarn one of higher elongation than that of the white yarn, and hence we conducted the following series of experiments.

The previously described starting material was used and by varying the spinning temperature in carrying out the melt-spinning of dope-dyed blue yarns multifilament yarns having various elongations were made. When these yarns were twisted together with white yarn, the results shown in Table II, below, were obtained.

40 Thus, it was found from the foregoing results that a uniform composite twisted yarn having few filament slacks and breaks could be obtained by raising the elongation of the dope-dyed blue yarn 3-9% above that of the white yarn. The difference in the inherent viscosity of the polymers of the several multifilament yarns before melt-spinning is not particularly a problem, since it can be compensated by adjustment of the spinning speed. Again, 45 the color of the dope-dyed yarn can be freely chosen, such as black, red, blue, brown, etc. Further, there is practically no difference in the Young's modulus of these drawn yarns as shown in Table IV, below.

TABLE IV

| Elongation, Percent | Young's modulus of dope-dyed yarn (kg./mm. <sup>2</sup> ) |       |       |       |       |
|---------------------|-----------------------------------------------------------|-------|-------|-------|-------|
|                     | Blue                                                      | Black | Red   | Green | Brown |
| 10                  | 1,350                                                     | 1,350 | 1,348 | 1,346 | 1,35  |
| 20                  | 1,301                                                     | 1,300 | 1,298 | 1,297 | 1,30  |
| 30                  | 1,282                                                     | 1,280 | 1,277 | 1,278 | 1,28  |

TABLE II

| Elongation of white yarn, percent | Elongation of dope-dyed blue yarn, percent | Difference in the percentages of the elongation | Number of spindles $\times$ time, hr. | Number of spindles in which slacks occurred | Number of spindles in which filament breaks occurred |
|-----------------------------------|--------------------------------------------|-------------------------------------------------|---------------------------------------|---------------------------------------------|------------------------------------------------------|
| 26                                | 27                                         | 1                                               | 150 $\times$ 24                       | 25                                          | 23                                                   |
| 26                                | 28                                         | 2                                               | 150 $\times$ 24                       | 15                                          | 11                                                   |
| 26                                | 29                                         | 3                                               | 150 $\times$ 24                       | 2                                           | 1                                                    |
| 26                                | 30                                         | 4                                               | 150 $\times$ 24                       | 1                                           | 2                                                    |
| 26                                | 31                                         | 5                                               | 150 $\times$ 24                       | 2                                           | 2                                                    |
| 26                                | 33                                         | 7                                               | 150 $\times$ 24                       | 1                                           | 1                                                    |
| 26                                | 35                                         | 9                                               | 150 $\times$ 24                       | 5                                           | 4                                                    |
| 26                                | 36                                         | 10                                              | 150 $\times$ 24                       | 21                                          | 15                                                   |
| 26                                | 37                                         | 11                                              | 150 $\times$ 24                       | 48                                          | 23                                                   |

Thus, it is apparent from the foregoing results that the occurrence of slacks and number of filament breaks are

75 Next it was found that the trouble (b) previously described, i.e., spottiness in the spoolly colored tones of

the woundup pirns, could be solved by adjusting the ratio of the denier of the white multifilament yarn used to that of the dope-dyed multifilament yarn used. In twisting together a dope-doped yarn containing 3.2% of black pigment (elongation 33%) and white yarn (elongation 28%), the denier ratio of two components were varied. One hundred and fifty ends of the so obtained yarns, after being wound up on pirns, were visually examined, with the results shown in Table V, below.

The method of examination consisted of visually examining the 150 pirns arranged side by side and picking up those which were either blacker or whiter than the standard, which was established for each denier ratio used. The numerals in the table indicate the number of pirns.

TABLE V

| Pirns                      | Denier ratio white:black |     |     |     |     |     |
|----------------------------|--------------------------|-----|-----|-----|-----|-----|
|                            | 1:3                      | 1:2 | 1:1 | 2:1 | 3:1 | 4:1 |
| Whiter than standard-----  | 6                        | 4   | 2   | 0   | 3   | 12  |
| Standard-----              | 132                      | 188 | 148 | 149 | 146 | 136 |
| Blacker than standard----- | 12                       | 8   | 0   | 1   | 1   | 2   |
| Variation (percent)-----   | 12.0                     | 8.0 | 1.2 | 0.7 | 2.4 | 9.3 |

Thus, it was found that when the denier ratio of white yarn to dope-dyed black yarn was within the range 1:1-3:1 an exceedingly stable color tone was exhibited.

It can be understood from the results of the various and numerous experiments hereinbefore presented that for obtaining sprinkly colored yarns which are even and without any spottiness in the sprinkly colored tone it is very important to specify the difference in elongation between the white and dope-dyed multifilament yarns as well as the denier ratio of the two yarns. The desired product of good quality cannot possibly be obtained by ignoring these two factors and just twisting the two multifilament yarns together. Although the aforementioned experiments were those carried out on the polyester type multifilament yarn, similar results are also obtained with respect to the other synthetic fibers, such, for example, as the polyamide, polyacrylonitrile and polyolefin type multifilament yarns. By knitting or weaving the so obtained sprinkly colored yarn, fabrics having a highly desirable sprinkly colored pattern are obtained. When this type of yarn or fabric is further overdyed, a sprinkly colored fibrous material of the desired tone can be obtained in accordance with the dyestuff used.

While the description given hereinbefore has concerned the twisting together of a white multifilament yarn and a dope-dyed multifilament yarn, we found that entirely identical conditions can be applied when twisting together two classes of white multifilament yarns whose dyeability differs. Thus, when an undrawn synthetic multifilament yarn of low dyeability and an undrawn synthetic multifilament yarn of higher dyeability are gathered together, drawn and twisted together, a yarn which can be dyed an even sprinkly colored pattern is made without appearance of slacks and breaks in the filaments provided that the yarns are chosen so that the elongation of the latter is 3-9% greater than that of the former and the denier ratio of the former to the latter is 1:1-3:1. When so obtained yarn or the fabrics knitted or woven therefrom are dyed using the conventional dyeing methods, sprinkly colored fibrous materials of the desired tones can be obtained.

In general, as the synthetic fiber of low dyeability, filaments of homopolymers are used, whereas as the synthetic fiber of high dyeability, filaments of copolymers, which have been prepared to enhance the dyeability, are used. Various fiber-forming copolymers, which have been prepared for enhancing the dyeability, are widely known. The comonomeric components used for making this type of copolymer include, in the case of the polyester type, such, for example, as adipic acid, sebacic acid, o-phthalic acid, isophthalic acid, sodium-5-sulfoisophthalate, polyethylene glycol, propylene glycol, polypropylene glycol, polypropylene glycol ethylene oxide addition product, and others; in the case of the acrylonitrile type, such, for

example, as styrene sulfonic acid, sodium styrene sulfonate and others; in the case of the polyolefin type, such, for example, as the vinyl monomers as vinyl pyridine, vinyl carbazole, vinyl quinoline, acrylonitrile, methyl acrylate, methyl methacrylate and vinyl acetate.

According to this invention, excellent sprinkly colored yarn, which had hitherto been unobtainable, can be readily obtained from two classes of undrawn multifilament yarns, using a single drawing and spinning machine.

For a better understanding of this invention, the following nonlimitative examples are given.

## EXAMPLE 1

15 Polyethylene terephthalate containing 1% titanium dioxide was melt-spun at a spinning temperature of 298° C. and a spinning speed of 1200 meters per minute and a white undrawn multifilament yarn of 175 total denier-24 filaments was obtained. On the other hand a dope-dyed black undrawn multifilament yarn of 70 total denier-8 filaments was made by melt-spinning polyethylene terephthalate containing 3.2% of carbon black at a spinning temperature of 286° C. and a spinning speed of 700 meters per minute. These two yarns were gathered together and were drawn 3.5X (the elongation after drawing was 28% for the former and 33% for the latter) and twisted together using a conventional drawing and spinning machine to obtain 150 ends of a 70D-32F yarn. The rate of occurrence of slacks was 1.3% and the rate of occurrence of filament breaks was 0%. The sprinkly colored pattern of black and white was very evenly distributed over the whole of the yarn.

Control.—A dope-dyed black yarn made in the same manner except that it was melt-spun at a spinning speed of 900 meters per minute had an elongation which showed hardly any difference from that of the aforesaid white yarn. When these two yarns were drawn and twisted together in similar manner, the rate of occurrence of slacks of 150 ends of the yarn was 15% while the rate of filament breaks was 7%. Furthermore, the sprinkly colored pattern was not as even as that obtained in the foregoing example.

## EXAMPLE 2

45 150 ends of a 60D-30F sprinkly colored yarn were prepared by drawing and twisting together a white polyethylene terephthalate multifilament yarn containing 4.1% of titanium dioxide (40D-18F, tenacity 5.0 g./d., elongation 27%) and a dope-dyed blue polyethylene terephthalate multifilament yarn containing 6.3% of Phthalocyanine Blue (20D-12F, tenacity 4.8 g./d., elongation 33%). The so obtained yarn was then processed with a false twisting machine CS-9R and knitted into a jersey. When the irregularity of the color tone was examined, it was only 0.7%.

50 Control.—When 150 ends of sprinkly colored yarns were prepared by drawing and twisting together the aforesaid white and dope-dyed blue yarns with the denier ratio of the former to the latter being 20 deniers to 40 deniers and thereafter the color tone irregularity was checked by the same method, there were present 12 ends (8%) which were irregular.

## EXAMPLE 3

55 The yarn obtained in Example 1 was processed with a false twisting machine CS-9R and then made into a jersey. When this was overdyed by the carrier dyeing method using the commercially available disperse dye Eastman Polyester Red, the white yarn was dyed red to yield readily a sprinkly colored pattern of red and black.

## EXAMPLE 4

60 The yarn obtained in Example 2 was processed and then knitted into a jersey, as described in Example 3. When this jersey was dyed using the commercially avail-

able disperse dye Amacron Blue, a sprinkly colored pattern of light and deep blue tones was obtained.

EXAMPLE 5

A 157.5 denier undrawn polyethylene terephthalate yarn of 12 filaments and a 105 denier undrawn yarn of 12 filaments of copolymeric polyethylene terephthalate containing 5 mol percent of sebacic acid (based on the dimethyl terephthalate) were drawn and twisted together at a drawing speed of 435 meters per minute and a draw ratio of 3.5 $\times$  (the tenacity elongation and shrinkage after drawing were 4.9 g./d., 29% and 7% for the former and 4.5 g./d., 34% and 9% for the latter) to obtain a 75D-24F drawn yarn. When this yarn was rewound with a cheese winder to a softness equalling a rubber hardness of 40 degrees and the cheese was dyed for 90 minutes at 100° C., a bath ratio 1:50 and 2% O.W.F., using the commercially available dyestuff Cibacet Blue 2R (C.I. 61110), a sprinkly colored yarn of evenly dyed tones of deep and light blue was obtained, the copolymeric yarn being dyed deep and the common yarn being dyed light.

EXAMPLE 6

The yarn obtained in Example 5, but before dyeing, was used and a tafetta fabric was woven. When this was dyed for 20 minutes at 100° C., a bath ratio 1:100 and 1% O.W.F., using the commercially available dyestuff Fast Green 3B (C.I. 55060), an evenly dyed sprinkly colored fabric having a pattern of deep and light green tones was obtained.

We claim:

1. A method of producing a sprinkly colored yarn which comprises gathering an undrawn synthetic multifilament yarn (A) and an undrawn dope-dyed synthetic multifilament yarn (B); drawing the gathered yarns so that the elongation of (B) is 3-9% greater than that of (A) and the denier ratio of (A) to (B) is between 1:1 and 3:1; and thereafter twisting the drawn yarns together.

2. A method of producing a sprinkly colored yarn which comprises gathering an undrawn synthetic multifilament yarn (A) and an undrawn dope-dyed synthetic multifilament yarn (B) of higher dyeability than that of synthetic multifilament yarn (A); drawing the gathered yarns so

that the elongation of (B) is 3-9% greater than that of (A) and the denier ratio of (A) to (B) is between 1:1 and 3:1; and thereafter twisting the drawn yarn together.

3. A method of producing a fibrous product having a sprinkly colored pattern which comprises over-dyeing the yarns obtained by the method of claim 1.

4. A method of producing a fibrous product having a sprinkly colored pattern which comprises dyeing the yarn obtained by the method of claim 2.

5. A method of producing a fibrous product having a sprinkly colored pattern which comprises making a fabric from the yarns obtained by the method of claim 1 and subsequently overdyeing said fabric.

10 6. A method of producing a fibrous product having a sprinkly colored pattern which comprises making a fabric from the yarns obtained by the method of claim 2 and subsequently dyeing said fabric.

References Cited

UNITED STATES PATENTS

|           |         |                              |
|-----------|---------|------------------------------|
| 2,278,888 | 4/1942  | Lewis.                       |
| 2,461,094 | 2/1949  | Taylor.                      |
| 2,805,465 | 9/1957  | Miller ----- 57-140 XR       |
| 2,904,953 | 9/1959  | Groombridge et al. 57-140 XR |
| 3,022,132 | 2/1962  | Shaw ----- 264-290 XR        |
| 3,053,604 | 9/1962  | Womble ----- 28-75 XR        |
| 3,061,998 | 11/1962 | Bloch ----- 57-140           |
| 3,137,989 | 6/1964  | Fior et al. ----- 57-140     |
| 3,375,651 | 4/1968  | Greeson ----- 28-75 XR       |

FOREIGN PATENTS

|           |         |                |
|-----------|---------|----------------|
| 719,046   | 10/1965 | Canada.        |
| 1,338,199 | 11/1962 | France.        |
| 1,423,757 | 11/1965 | France.        |
| 1,059,567 | 2/1967  | Great Britain. |

JORDAN FRANKLIN, Primary Examiner

WERNER H. SCHROEDER, Assistant Examiner

40 U.S. Cl. X.R.

8-14, 21; 28-75; 57-140, 157

UNITED STATES PATENT OFFICE  
CERTIFICATE OF CORRECTION

Patent No. 3,468,121 Dated September 23, 196

Inventor(s) Hirotaka Nakashima et al.

It is certified that error appears in the above-identified patent and that said Letters Patent are hereby corrected as shown below:

Column 4, (Table IV), lines 56, 57 and 58 (under last column of table entitle "Brown");

line 56 should read -- 1,354-- in lieu of "1,35".

line 57 should read -- 1,305 -- in lieu of "1,30".

line 58 should read -- 1,286 -- in lieu of "1,28".

Signed and sealed this 31st day of August 1971.

(SEAL)

Attest:

EDWARD M. FLETCHER, JR.  
Attesting Officer

ROBERT GOTTSCHALK  
Acting Commissioner of Paten